

## UNITED STATES PATENT OFFICE.

THOMAS P. SHIELDS, OF NEW YORK, N. Y., ASSIGNOR TO SHIELDS & MOORE, A FIRM CONSISTING OF THOMAS P. SHIELDS AND G. A. MOORE, OF NEW YORK, N. Y.

## GOLD ALLOY.

No Drawing.

Application filed May 15, 1924. Serial No. 713,617.

*To all whom it may concern:*

Be it known that I, THOMAS P. SHIELDS, a citizen of the United States, residing at New York, N. Y., have invented certain new and useful Improvements in Gold Alloys, of which the following is a specification.

The present invention relates to the production of a white gold alloy and has for its object to produce an alloy as above referred to which is easy to work by the tools ordinarily used by goldsmiths, engravers and the like, it is capable of taking a very high polish, capable of withstanding the influence of the atmosphere, and which will be economical to manufacture. In the preferred form of the invention the color of the so-called "white gold" has a somewhat bluish cast, the alloys produced in accordance with the present invention are very desirable for manufacturing jewelry and for similar uses, although it will be understood that the alloy when produced can be used as a substitute for pure gold in many other arts besides the manufacture of jewelry.

The fineness of the gold alloy can be varied considerably and for making jewelry, I find it advisable to use an alloy of about 18 k. However, owing to the conditions in the jewelry trade, it is sometimes advisable to produce alloy in accordance with the present invention ranging from about 17½ to 19½ k.

In accordance with the present invention, the major constituent of the alloy is gold, and for adjusting the degree of fineness of the alloy, copper can be added, in amount up to 10% and the addition of this amount of copper does not have any very marked influence upon the properties of the final alloy, (such as the ease of working, hardness, etc.) other than the fineness of the product.

For making a suitable alloy I may use 75 parts of gold, 18 parts of iron, 7 parts of nickel, and ½ part of manganese or silicon, and may also use with the above as a diluent, from 5 to 10% of copper. These proportions are given by way of example, and can be varied. This base can subsequently be melted and gold or copper then added to adjust the fineness as desired. It is not necessary to add any other noble metals to the alloy.

Heretofore in the manufacture of white

gold it has been proposed to use palladium or zinc, or both of these, it has also been proposed to use copper as a diluent, for reducing the fineness of the alloy. In accordance with the present invention I use iron instead of palladium, which substitution I find to be entirely feasible and the substitution of iron greatly reduces the cost of the final alloy. Zinc has heretofore been used in alloys of this general character, but zinc makes the alloy too hard and difficult to work with ordinary tools, such as are used in the art, in working pure gold, or gold-copper alloy.

I have above referred to a specific formula, which has been found to produce very satisfactory results. I will say, however, that the proportions can be substantially varied, thus the gold may be from 72 to 82%, the iron from 10 and 20%, the nickel between 5 and 20% and the manganese or silicon between ½ and 5%, of the total alloy.

The function of the manganese or silicon is that of a deoxidizer, and it is to be noted that both of these elements form relatively stable oxids of the type  $AO_2$ .

While of course ordinarily iron would be used which is entirely free from rust, and all the metals substantially free from oxids, it is found advisable to use, in all cases, a small amount of the deoxidizer, such as manganese or silicon, which elements unite with any oxide present in the iron, nickel or copper, and also they unite with an oxide or oxygen taken up by the constituents of the alloy during the making of the alloy.

I call attention to the fact that the alloy in its preferred form does not contain any other noble metals besides gold, thereby effecting a great saving in the production of white gold. Thus the alloy does not contain palladium or other metals of that group, all of which are extremely expensive.

As a preferred mode of making the alloy, to which the invention is not restricted, the following is given:—

The iron, nickel and manganese or silicon are melted together, say in a crucible provided with a cover, in the proportions of, say 70 to 28 to 2. When a quiet molten liquid is produced, this can be "granulated" by being poured into cold water or it may be

cast into an ingot and rolled out into a sheet, say 0.02 inch thick, and cut up into small pieces. The comminuted metal is then mixed with metallic gold and copper and 5 melted in a covered graphite crucible, and then cast into ingots to be suitably worked up.

I claim:

1. An alloy containing not substantially 10 below 70% of gold, much smaller but substantial proportions of both iron and of nickel, the two latter amounting to not less than 15% of the alloy, and the iron being over half the amount of nickel, and a still 15 smaller amount of a deoxidizer, such deoxidizer being a solid element which readily forms a solid oxid of the type  $AO_2$ , such alloy being of a whitish color, and such alloy being free from other noble metals.
2. An alloy containing not substantially 20 below 70% of gold, much smaller but substantial proportions of both iron and of nickel, the two latter amounting to not less than 15% of the alloy, and the iron being 25 over half the amount of nickel, and a still smaller amount of a deoxidizer, such deoxidizer being a solid element which readily forms a solid oxid of the type  $AO_2$ , such alloy being of a whitish color, such alloy 30 also containing copper in substantial amount but not above 10%.

3. An alloy having substantially the following analysis:

|        | Parts.      |
|--------|-------------|
| Gold   | 72 to 82 35 |
| Iron   | 10 to 20    |
| Nickel | 5 to 20     |

Deoxidizer in the form of a solid element that readily forms a solid oxid of the type  $AO_2$ , 0.5 to 5 40

Copper In appreciable amount up to 10 4. An alloy having the following analysis:

|        | Parts.  |
|--------|---------|
| Gold   | 75      |
| Iron   | 18 45   |
| Nickel | about 7 |

Deoxidizer in the form of a solid element that readily forms a solid oxid of the type  $AO_2$ , 0.5

Copper 5 to 10 50

5. An alloy having substantially the following analysis:

|      | Parts.      |
|------|-------------|
| Gold | 72 to 82    |
| Iron | 10 to 20 55 |

Nickel 5 to 20

Deoxidizer in the form of a solid element that readily forms a solid oxid of the type  $AO_2$ , 0.5 to 5

In testimony whereof I affix my signature.

THOMAS P. SHIELDS.